# EUROPEAN PATENT APPLICATION

(11) **EP 0 377 276 A1**
(43) Date of publication of application: **11.07.1990**
(21) Application number: 89311215.1
(22) Date of filing: 31.10.1989
(51) Int. Cl.: C25C 7/02, C25D 17/10

(54) **Corrosion resistant electrode for electrochemical use**

(30) Priority: 31.10.1988 ZA 888152
(71) Applicant: ZIMCO INDUSTRIES (PROPRIETARY) LIMITED, Sandton City Sandton Transvaal (ZA)
(72) Inventor: Thom, Michael John, Bushyvales South Coast Natal (SA)
(74) Representative: White, Martin David

(57) **Abstract**

An electrode is formed by electrodepositing on calcium/lead alloy electrode body (14) a lead/mixture (22) with a grain size which is finer than the grain size of the electrode body. The electrode's resistance to corrosion is thereby enhanced.

## Description

### BACKGROUND OF THE INVENTION

This invention relates generally to an electrode and more particularly is concerned with an electrode which is corrosion resistant.

The invention is also concerned with a method of making a corrosion resistant electrode. The method may be applied in the manufacture of new electrodes and to the refurbishing or re-conditioning of corroded electrodes and the scope of the invention is to be interpreted in this sense.

The surface of an electrode, during use, tends to corrode because of the migration of ions from the electrode surface. This effect is particularly pronounced in certain electrolytic and metallurgical processes.

Once electrode corrosion has commenced it tends to accelerate with time because most electrolytic and metallurgical processes based on ion migration and using electrodes, such as electroplating, electrodeposition and electrowinning, require surface reactions. With the erosion of the electrode surface cell environments are presented with increased electrode surfaces which result in increasing ion losses from the electrode.

Electrode corrosion decreases the life of the electrode, leads to contamination of the electrolyte in which the electrode is used, and degrades the purity of the material produced in the electrolytic process.

### SUMMARY OF THE INVENTION

The invention is concerned, in the first instance, with an improved electrode.

The invention provides an electrode which includes an electrode body which is formed from a first material, and at least one outer layer of a second material on at least a portion of the electrode body, the second material having a grain size which is finer than the grain size of the first material.

Preferably the entire surface of the electrode body, which reacts in the electrolytic process, is covered with a layer of the second material.

The grain size of the second material may increase in a direction away from the electrode body. Alternatively the grain size of the second material may decrease in a direction away from the electrode body.

It is possible to form the electrode with a plurality of the said outer layers, one over the other on the electrode body. Within each layer the grain size is finer than the grain size of the first material. It is not necessary however that the grain size in each layer is the same as in any other layer. Thus the grain size in each layer, the thickness of each layer, and the material from which each layer is formed, may be varied to achieve different properties.

The first material may be the same as the second material and, in this case, the first material may be of a lower grade than the second material. Under these circumstances the second material will normally be more expensive than the first material. More generally, however, the first material is different from the second material.

In the latter instance the first material may comprise aluminium of a calcium/lead alloy and the second material may comprise a silver/lead alloy mixture.

If the first material is aluminium then once the aluminium has been cleaned it may be coated with silver or gold in an inert atmosphere, or using any other technique, or be tinned with a tin/lead alloy using a suitable flux. The silver/lead alloy is then formed over this coating.

The invention also extends to a method of making an electrode which includes the step of forming on an electrode body of a first material at least one layer of a second material with the grain size of the second material being finer than the grain size of the first material.

As has been indicated a plurality of the said layers may be formed on the electrode body.

The layer of the second material may be formed by any suitable process and preferably is formed by a process selected from the following: electrophoresis, electrostatic spraying, electrodeposition, and electrocoating.

The method may include the prior step of cleaning a surface of the electrode body, on which the layer is formed, by a process selected from the following: sand blasting, electropolishing, and exposure to a suitable reagent. In the last mentioned case use may be made of dilute nitric acid or acetic acid solution. If the electrode body is aluminium then it may be cleaned with NaOH or NaCO₃.

The two materials may be the same, or different. The first material may for example be a calcium/lead alloy or aluminium and in the latter case the aluminium could be coated with a silver or gold, or a tin/lead alloy, using any suitable technique. The layer of the second material is then formed thereon.

In one form of the invention the layer of the second material is formed by electrodeposition in an electrolysis tank and the grain size, and the thickness, of the layer of the second material are controlled by at least one process selected from the following: varying the density of an electric current in the tank, the period of time for which the current flows in the tank, and adding any suitable optical brightener to the electrolyte in the tank. In the last mentioned case the optical brightener may for example be an aldehyde or a ketone, based glue, or any other based-glue brightener. This may be added to the electrolyte in the range of from 0 to 0,3% by weight. The addition of the optical brightener generally leads to a reduction in the coarseness of the grain size. As has been indicated the grain size can also be varied by controlling the current density in the electrolyte. The current density can vary from between 0,5 amps per square decimetre to 0,05 amps per square decimetre. The variation may be continuous or stepped or follow any other suitable pattern. An increase in current density leads to a decrease in the coarseness of the grain size.

The thickness of each layer may be controlled by controlling the time period for which current flows in the electrolyte. The thickness of each layer may vary according to requirement and may for example lie in the ranged from 1 to 10 microns.

In one form of the invention the first material is a calcium/lead alloy, the electrolysis tank contains, as electrolyte, sodium hydroxide in solution with sodium cyanide, or potassium hydroxide in solution with potassium cyanide, or a mixture thereof, lead hydroxide and silver cyanide, and a layer of lead and silver is deposited on the electrode body.

It is to be noted that, as used herein, the term "electrode body" includes a newly formed electrode body and the body of an electrode which is to be re-conditioned or refurbished.

### BRIEF DESCRIPTION OF THE DRAWINGS

The invention is further described by way of example with reference to the accompanying drawings in which:
Figure 1 schematically depicts the manner in which an electrode is formed in accordance with the invention, and
Figure 2 is an enlarged cross-sectional view of portion of an electrode according to the invention.

### DESCRIPTION OF PREFERRED EMBODIMENT

Figure 1 of the accompanying drawings illustrates an electrode tank 10 which contains an electrolyte 12 which comprises sodium hydroxide in solution with sodium cyanide, or potassium hydroxide in solution with potassium cyanide, or a mixture thereof, lead hydroxide and silver cyanide.

A calcium/lead alloy electrode body 14, of a desired shape and size, is formed in a conventional way and thereafter is cleaned by sand blasting, electropolishing, or by dipping an electrode body in a suitable reagent such as a dilute nitric acid or acetic acid solution. The electrode body 14 is placed in the tank and connected to one terminal of a controllable power supply 16.

Connected to a remaining terminal of the voltage supply is a lead sheet 18 which contains from 4% to 7% silver. The exact amount of silver is varied according to requirement so that a desired percentage of silver, say 5%, is deposited on the electrode body.

The power supply 16 is under the control of a control unit 20 by means of which the duration, amplitude and waveform of the current which passes between the electrode body 14 and lead sheet 18, can be controlled. It is also possible to vary the spacing between the body 14 and the lead sheet thereby to control the amplitude of the current.

When current flows in the electrolyte 12 electrodeposition of lead and silver ions takes place from the lead sheet 18 to the electrode body 14. A layer of lead and silver is thereby deposited on the electrode body.

Figure 2 shows in cross-section portion of the electrode body 14 with a lead/silver layer 22 deposited thereon.

The grain size of the particles in the lead/silver layer 22 is, in accordance with the invention, finer than the grain size of the particles in the calcium/lead electrode body 14. The grain size of the deposited lead/silver ions can be varied in several ways. For example the current density in the tank 10 can be varied from between 0,5 amps per square decimetre to 0,05 amps per square decimetre. The variation may be continuous or stepped or follow any other suitable waveform. Increasing the current density leads to a reduction in grain size. In this way the sizes of the grains in the deposited layer 22 can be carefully controlled.

The thickness of the layer 22 can be controlled by varying the time period for which current flows between the electrode body 14 and the lead sheet 18. Consequently by careful control of the current density and the period for which the current flows the grain size and the thickness of the layer 22 can be controlled according to requirement. The thickness of the layer 22 may vary according to need and generally is in the range of from 1 to 10 microns.

It is to be noted that it is also possible to vary the grain size of the deposited ions by the addition of an optical brightener which may be glue-based, such as an aldehyde or ketone base glue, to the electrolyte. This may be added to the electrolyte in the range of from 0 to 0,3% by weight. An increase in the amount of optical brightener leads to a reduction in the grain size of the deposited ions.

The aforementioned processes for varying grain size may, if required, be employed singularly or in combination.

The formation of the electrode has been described with reference to a single electrode body 14, and a single lead sheet 18. A plurality of these compounds can simultaneously be used in a single electrolytic tank, all connected to the power supply 16. The provision of a suitable power supply 16, and the control unit 20, lies within the scope of those skilled in the art and consequently these aspects are not further described herein.

It is also possible to form a plurality of successive layers 22A, shown in dotted outline, on the electrode body 14. This may be done, for example, by changing the composition of the electrolyte in the tank 10 or by moving the electrode body through a series of electrolysis tanks each of which each contains an appropriate electrolyte.

Within the or each layer which is deposited on the electrode body the grain size is, as has been pointed out, finer than the grain size of the calcium lead body. Notwithstanding this characteristic the grain size in the or each layer may vary and become progressively coarser or finer with increasing distance from the electrode body 14.

The electrode produced in accordance with the aforementioned method exhibits an increased resistance to corrosion. The exact reason for this is not known but it is believed that this is due to the fact that the surface of the electrode, before the deposition of the layer, is considerably indented and consequently the ions which are deposited progressively fill up the indentations so that the electrode ultimately presents to the electrolyte, in an actual metallurgical operation, a smoother and less indented surface which means that the surface area over which corrosion can take place is reduced.

## Claims

1. An electrode which includes an electrode body (14) which is formed from a first material, and which is characterized by at least one outer layer (22) of a second material on a least a portion of the electrode body, the second material having a grain size which is finer than the grain size of the first material.

2. An electrode according to claim 1 characterized in that the grain size of the second material increases in a direction away from the electrode body.

3. An electrode according to claim 1 characterized in that the grain size of the second material decreases in a direction away from the electrode body.

4. An electrode according to claim 1, 2 or 3 which is characterized in that it includes a plurality of the said outer layers (22), one over the other on the electrode body.

5. An electrode according to claim 4 characterized in that each outer layer (22) is of a different material.

6. An electrode according to any of claims 1 to 4 characterized in that the first material is different from the second material.

7. An electrode according to any one of claims 1 to 4 characterized in that the first material is the same as the second material.

8. An electrode according to claim 7 characterized in that the first material is of a lower grade than the second material.

9. An electrode according to claim 6 characterized in that the first material is a calcium/lead alloy and the second material is a silver/lead alloy.

10. An electrode according to claim 6 characterized in that the first material is aluminium and the second material is a silver/lead alloy.

11. A method of making an electrode which is characterized by the step of forming on an electrode body (14) of a first material at least one layer (22) of a second material with the grain size of the second material being finer than the grain size of the first material.

12. A method according to claim 11 characterized in that the layer of the second material is formed by a process selected from the following: electrophoresis, electrostatic spraying, electrodeposition, and electro-coating.

13. A method according to claim 11 or 12 which is characterized by the prior step of cleaning the surface of the electrode body (14), on which the layer is formed, by a process selected from the following: sand blasting, electro-polishing, and exposure to a suitable reagent.

14. A method according to claim 12 or 13 characterized in that the layer (22) of the second material is formed by electrodeposition in an electrolysis tank (10) and which includes the step of controlling the grain size, and the thickness, of the layer of the second material by at least one process selected from the following: varying the density of electric current in the tank, the period of time for which the current flows in the tank, and adding an optical brightener to the electrolyte in the tank.

15. A method according to claim 14 characterized in that the first material is a calcium/lead alloy, the electrolysis tank (10) contains, as electrolyte (12), sodium hydroxide in solution with sodium cyanide, or potassium hydroxide in solution with potassium cyanide, or a mixture thereof, lead hydroxide and silver cyanide, and a layer (22) of lead and silver is electrodeposited on the electrode body.
